



US011525265B2

(12) **United States Patent**  
**Johnson et al.**

(10) **Patent No.:** **US 11,525,265 B2**  
(45) **Date of Patent:** **Dec. 13, 2022**

(54) **PERMEABLE WATER RESISTIVE ROOF  
UNDERLAYMENT**

(71) Applicant: **VAPROSHIELD LLC**, Gig Harbor, WA (US)

(72) Inventors: **Philip L. Johnson**, Spring Lake, MI (US); **Kevin D. Nolan**, Seattle, WA (US); **Daniel Bess**, Newbury, OH (US); **Adrian deKrom**, Cardon, OH (US)

(73) Assignee: **VaproShield, LLC**, Gig Harbor, WA (US)

(\*) Notice: Subject to any disclaimer, the term of this patent is extended or adjusted under 35 U.S.C. 154(b) by 43 days.

(21) Appl. No.: **16/602,328**

(22) Filed: **Sep. 18, 2019**

(65) **Prior Publication Data**

US 2020/0087916 A1 Mar. 19, 2020

**Related U.S. Application Data**

(60) Provisional application No. 62/732,908, filed on Sep. 18, 2018.

(51) **Int. Cl.**

**E04D 5/10** (2006.01)  
**E04D 11/02** (2006.01)

(52) **U.S. Cl.**

CPC ..... **E04D 5/10** (2013.01); **E04D 11/02** (2013.01)

(58) **Field of Classification Search**

CPC ..... E04D 5/10; E04D 11/02; E04D 12/002  
See application file for complete search history.

(56)

**References Cited**

U.S. PATENT DOCUMENTS

|             |         |              |
|-------------|---------|--------------|
| 2,140,026 A | 12/1938 | Edward       |
| 3,440,185 A | 4/1969  | Hanley       |
| 3,445,272 A | 5/1969  | Newton, Jr.  |
| 3,539,388 A | 11/1970 | Shu-Tung     |
| 3,979,867 A | 9/1976  | Sowinski     |
| 4,098,044 A | 7/1978  | Slavik       |
| 4,163,822 A | 8/1979  | Walter       |
| 4,252,590 A | 2/1981  | Rasen et al. |

(Continued)

FOREIGN PATENT DOCUMENTS

|    |         |        |
|----|---------|--------|
| CA | 2843707 | 2/2017 |
| CA | 2887478 | 1/2018 |

(Continued)

OTHER PUBLICATIONS

British Board of Agreement, Tyvek® Supro Roof Tile Underlayment for Use in Warm Non-Ventilated and Cold Ventilated Roofs, Certificate No. 08/4548, Apr. 8, 2008.

(Continued)

*Primary Examiner* — Callie E Shosho

*Assistant Examiner* — Bethany M Miller

(74) *Attorney, Agent, or Firm* — Janeway Patent Law PLLC; John Janeway

(57) **ABSTRACT**

The present invention relates to a water resistant, UV resistant, vapor permeable, air barrier roofing underlayment assembly for use on flat or low sloped roofs comprising a substrate of permeable polyester, a permeable copolymer acrylate coating bonded to the permeable polyester substrate and a pressure sensitive permeable copolymer adhesive secured to the acrylate coating. The permeable coating is a copolymer including a primary polymer of n-butyl acrylate and contains carbon black.

**16 Claims, 1 Drawing Sheet**



# US 11,525,265 B2

Page 2

| (56) <b>References Cited</b> |         |                       |                                                                                                                                                                                                                                                                                       |                    |                 |              |
|------------------------------|---------|-----------------------|---------------------------------------------------------------------------------------------------------------------------------------------------------------------------------------------------------------------------------------------------------------------------------------|--------------------|-----------------|--------------|
| U.S. PATENT DOCUMENTS        |         |                       |                                                                                                                                                                                                                                                                                       |                    |                 |              |
| 4,315,392 A                  | 2/1982  | Sylvest               | 2008/0268224 A1                                                                                                                                                                                                                                                                       | 10/2008            | Kim             |              |
| 4,655,210 A                  | 4/1987  | Edenbaum              | 2009/0047465 A1                                                                                                                                                                                                                                                                       | 2/2009             | Zafiroglu       |              |
| 4,764,412 A                  | 8/1988  | Burns                 | 2009/0288358 A1                                                                                                                                                                                                                                                                       | 11/2009            | Snyder          |              |
| 4,815,963 A                  | 3/1989  | Berkhout              | 2011/0185666 A1                                                                                                                                                                                                                                                                       | 8/2011             | Russell         |              |
| 4,851,272 A                  | 7/1989  | Knox, III             | 2011/0312240 A1 *                                                                                                                                                                                                                                                                     | 12/2011            | Amthor          | C09D 133/066 |
| 5,099,627 A                  | 3/1992  | Coulton et al.        |                                                                                                                                                                                                                                                                                       |                    |                 | 442/327      |
| 5,425,672 A                  | 6/1995  | Rotter                | 2012/0244340 A1 *                                                                                                                                                                                                                                                                     | 9/2012             | Peng            | E04D 5/06    |
| 5,598,673 A                  | 2/1997  | Atkins                |                                                                                                                                                                                                                                                                                       |                    |                 | 428/327      |
| 5,617,687 A                  | 4/1997  | Bussey, Jr.           | 2013/0052401 A1                                                                                                                                                                                                                                                                       | 2/2013             | Snyder          |              |
| 5,709,651 A                  | 1/1998  | Ward                  | 2015/0024159 A1                                                                                                                                                                                                                                                                       | 1/2015             | Bess et al.     |              |
| 5,960,595 A                  | 10/1999 | McCorsley, III et al. | 2015/0136207 A1 *                                                                                                                                                                                                                                                                     | 5/2015             | Giron           | B62D 29/043  |
| 5,973,015 A                  | 10/1999 | Coronado et al.       |                                                                                                                                                                                                                                                                                       |                    |                 | 136/251      |
| 5,993,927 A                  | 11/1999 | Sugita et al.         | 2015/0307751 A1 *                                                                                                                                                                                                                                                                     | 10/2015            | Eckhardt        | B32B 27/302  |
| 6,131,353 A                  | 10/2000 | Egan                  |                                                                                                                                                                                                                                                                                       |                    |                 | 428/41.8     |
| 6,284,368 B2                 | 9/2001  | Muta                  | 2016/0024782 A1                                                                                                                                                                                                                                                                       | 1/2016             | Bess et al.     |              |
| 6,316,016 B1                 | 11/2001 | Iwakawa               | 2017/0044404 A1                                                                                                                                                                                                                                                                       | 2/2017             | Yamamoto et al. |              |
| 6,594,965 B2                 | 7/2003  | Coulton               | 2017/0174952 A1                                                                                                                                                                                                                                                                       | 6/2017             | Bess et al.     |              |
| 6,804,922 B1                 | 10/2004 | Egan                  | 2018/0237662 A1 *                                                                                                                                                                                                                                                                     | 8/2018             | Widenbrant      | B32B 7/06    |
| 6,927,267 B1                 | 8/2005  | Varela de la Rosa     | FOREIGN PATENT DOCUMENTS                                                                                                                                                                                                                                                              |                    |                 |              |
| 6,938,383 B2                 | 9/2005  | Morris et al.         | EP                                                                                                                                                                                                                                                                                    | 0397554 B1         | 8/1994          |              |
| 7,117,649 B2                 | 10/2006 | Morris et al.         | EP                                                                                                                                                                                                                                                                                    | 0874099 A2         | 2/2001          |              |
| RE39,825 E                   | 9/2007  | Morris et al.         | FI                                                                                                                                                                                                                                                                                    | 116226 B           | 10/2005         |              |
| 7,488,523 B1                 | 2/2009  | Muncaster             | GB                                                                                                                                                                                                                                                                                    | 2473618            | 3/2011          |              |
| 7,617,638 B1                 | 11/2009 | Slama et al.          | JP                                                                                                                                                                                                                                                                                    | 07048554 A         | 2/1995          |              |
| 7,651,757 B2                 | 1/2010  | Jones et al.          | JP                                                                                                                                                                                                                                                                                    | H7-138539          | 5/1995          |              |
| 8,146,310 B2                 | 4/2012  | Keene                 | JP                                                                                                                                                                                                                                                                                    | 2001003025 A       | 1/2001          |              |
| 8,245,472 B2                 | 8/2012  | Keene                 | MX                                                                                                                                                                                                                                                                                    | PA03001867 A       | 6/2003          |              |
| 8,387,336 B2                 | 3/2013  | Coulton               | WO                                                                                                                                                                                                                                                                                    | 2006047130 A1      | 11/2006         |              |
| 8,549,806 B2                 | 10/2013 | Snyder                | WO                                                                                                                                                                                                                                                                                    | 2008067611 A1      | 6/2008          |              |
| 8,590,267 B2                 | 11/2013 | Jaffee                | WO                                                                                                                                                                                                                                                                                    | 2009/127819 A1     | 10/2009         |              |
| 9,286,577 B2                 | 3/2016  | Shofner et al.        | WO                                                                                                                                                                                                                                                                                    | WO-2009127819 A1 * | 10/2009         | B32B 23/08   |
| 9,453,337 B2                 | 9/2016  | Fritz                 | WO                                                                                                                                                                                                                                                                                    | 2010056372 A1      | 5/2010          |              |
| 9,783,980 B2                 | 10/2017 | Snyder et al.         |                                                                                                                                                                                                                                                                                       |                    |                 |              |
| 2002/0037956 A1 *            | 3/2002  | Avramidis             | OTHER PUBLICATIONS                                                                                                                                                                                                                                                                    |                    |                 |              |
|                              |         | C08L 2666/04          | Derwent Abstract of JP 2001-3025.                                                                                                                                                                                                                                                     |                    |                 |              |
|                              |         | 524/523               | Cosella-Dorken Products, Inc. Technical Data Sheet for Delta®-Fassade S and Delta®-Fassade S Plus UV, Dec. 21, 2011. Cosella-Dorken Products, Inc. Technical Data Sheet for Delta®-Vent S. E.I. du Pont De Nemours and Company, "DuPont Tyvek® Providing Protection in Construction". |                    |                 |              |
| 2002/0146953 A1              | 10/2002 | Lubker, II            | Irish Agreement Board, "DuPont Tyvek® Supro Vapour Permeable Roofing Underlays for Pitched Roofs", Certificate No. 04/0157, Nov. 2004.                                                                                                                                                |                    |                 |              |
| 2003/0232171 A1              | 12/2003 | Keith                 | British Board of Agreement, Tyvek® Supro Roof Tile Underlayment for Use in Warm Non-Ventilated and Cold Ventilated Roofs, Certificate No. 08/4548, Apr. 8, 2008.                                                                                                                      |                    |                 |              |
| 2004/0106346 A1              | 6/2004  | Zafiroglu             |                                                                                                                                                                                                                                                                                       |                    |                 |              |
| 2004/0180195 A1              | 9/2004  | Macuga                |                                                                                                                                                                                                                                                                                       |                    |                 |              |
| 2004/0237464 A1              | 12/2004 | Khan                  |                                                                                                                                                                                                                                                                                       |                    |                 |              |
| 2005/0000172 A1              | 1/2005  | Anderson              |                                                                                                                                                                                                                                                                                       |                    |                 |              |
| 2005/0014431 A1              | 1/2005  | Carmody et al.        |                                                                                                                                                                                                                                                                                       |                    |                 |              |
| 2005/0055983 A1              | 3/2005  | Tomes                 |                                                                                                                                                                                                                                                                                       |                    |                 |              |
| 2005/0214496 A1              | 9/2005  | Borenstein            |                                                                                                                                                                                                                                                                                       |                    |                 |              |
| 2006/0096218 A1              | 5/2006  | Johnson               |                                                                                                                                                                                                                                                                                       |                    |                 |              |
| 2006/0101758 A1              | 5/2006  | Egan                  |                                                                                                                                                                                                                                                                                       |                    |                 |              |
| 2006/0211781 A1              | 9/2006  | Strandburg            |                                                                                                                                                                                                                                                                                       |                    |                 |              |
| 2007/0212520 A1              | 9/2007  | Furumori et al.       |                                                                                                                                                                                                                                                                                       |                    |                 |              |
| 2008/0120935 A1              | 5/2008  | Lembo                 |                                                                                                                                                                                                                                                                                       |                    |                 |              |

\* cited by examiner

Fig. 1



Fig. 2



## PERMEABLE WATER RESISTIVE ROOF UNDERLayment

### RELATED APPLICATIONS

The present applications claims priority and benefits from U.S. provisional application Ser. No. 62/732,908 filed Sep. 18, 2018.

### STATEMENT REGARDING FEDERALLY SPONSORED RESEARCH OR DEVELOPMENT

None

### REFERENCE TO SEQUENCE LISTING, A TABLE OR A COMPUTER PROGRAM LISTING COMPACT DISC APPENDIX

None.

### BACKGROUND OF THE INVENTION

#### 1. Field of Invention

The present invention relates to a building construction membrane, and more particularly to a non-asphaltic roof underlayment that is vapor permeable, forms an air barrier, and is resistant to water and ultra-violet (UV) light. The underlayment can be a component of a roof assembly on both flat and low sloped roofs.

#### 2. Background of the Invention

In the roofing industry, a roofing underlayment is typically applied to a low slope roof to form a vapor and air barrier over which insulation and a roof cover is applied. A primary goal of the low slope roof underlayment is to stop vapor and air. However, in a number of applications, it is preferable to have vapor migration and stop air infiltration. The present invention is directed toward the latter application.

It is known in the prior art that flat or low-sloped roofs are often covered with top roofing membranes. Common among the membranes that have the mechanical properties needed to be technologically useful are thermoset membranes such as EPDM rubber and thermoplastic membranes such as PVC and TPO. These membranes typically contain carbon black, titanium oxide ( $TiO_2$ ) and/or other mineral fillers to add advantageous mechanical properties to the membranes.

In most cases, the roofing underlayment comprises a felt material composed of cellulose or glass fibers or a mixture thereof that is saturated with a bituminous material such as asphalt or pitch. Roofing underlays that are saturated with a bituminous material can be hazardous to manufacture due to the presence of a flammable bituminous material and can contribute to fire on a construction site or a finished roof assembly. Many of the asphaltic underlays available in the market tend to wrinkle after being applied to a roofing deck due to minor amounts of moisture. This is especially the case if the underlays are rained upon. Other common problems are underlayment blowing off due to wind. Another major deficiency of a roofing substrate of asphalt or bituminous material is that the material is non-renewable.

The roofing industry has also developed non-asphaltic, underlays which are butyl based. There are also other types of non-asphaltic membranes used as underlays such as polyethylene.

Currently, all of the commercial asphaltic and non-asphaltic underlays tend to be water-resistant but substantially non-breathable or with no permeability. That is, both asphaltic and non-asphaltic underlays do not allow water vapor to pass through it. As a result, the moisture from the interior of the roofing assembly is trapped in the roof composite of insulation and top roofing membranes and is unable to escape to the exterior atmosphere resulting in damage to the roof over a number of years. Furthermore, asphaltic membranes can degrade due to UV radiation from the sun.

U.S. Pat. No. 4,511,619 issued Apr. 16, 1985 discloses a sealing sheet for the building industry made up of at least one layer that contains filler such as carbon black mixed with an ethylene-propylene copolymer which has a reinforcing laminate in place. The reinforcing layer can be formed of a fabric, a mat, a knitted material, a non-woven material, a synthetic resin or a glass fiber.

U.S. Patent Application Publication Number 2014/0072751 published Mar. 13, 2014 discloses a single-ply polymer coated substrate with at least one adhesive layer for structural water proofing.

U.S. Pat. No. 8,309,211 issued Nov. 13, 2012 discloses a roofing underlayment substrate that is permeable transmitting water vapor at a minimum of 3 perms, water resistant and skid-resistant. The roofing underlayment includes a woven or non-woven substrate having at least one surface which includes a breathable thermoplastic film which also imparts water-resistant to the substrate.

U.S. Pat. No. 8,347,576 issued Jan. 8, 2013 discloses a single-ply mechanically embossed roofing membrane in roll form for use in commercial application on flat and low pitched roofs.

None of the aforementioned references appear to be permeable to allow meaningful transmissions of water vapor or are designed to be UV resistant or attempt to prevent or preclude mold, mildew, rot from forming on a substantially flat roof structure.

These teachings do not aid in the resolution of a number of practical difficulties that are resolved by the present invention.

In view of the drawbacks mentioned above with prior art non-asphaltic underlays, there is a need for providing a non-asphaltic self adhering roofing underlayment that is a breathable air barrier thereby allowing moisture in the form of water vapor to escape from inside the roof assembly, while preventing water vapor moisture from destroying the roofing composite of insulation and roofing membrane. In addition, UV-resistance is a highly desirable property of an underlayment.

### SUMMARY OF THE INVENTION

The present invention is directed towards a flat roofing self-adhering underlayment that is water resistive, UV resistant and a vapor permeable air barrier. The roofing underlayment is a polyester substrate which is coated with a foamed n-butyl acrylate copolymer containing carbon black and cured to maintain air bubble pores in place. A permeable pressure sensitive copolymer adhesive coating having a back bone of n-butyl acrylate, 2-ethylhexyl acrylate and vinyl acetate is foamed and coated over the n-butyl acrylate copolymer coating, bonding to the coating with a reduction in tackiness in the adhesive which may eliminate the need for a slip sheet in some usages. After curing, the pressure sensitive adhesive, coating and substrate is laminated.

In one particular embodiment, a single-ply permeable polyester substrate has a permeable acrylate coating on the bottom side of the base substrate and a permeable adhesive applied over the acrylate coating.

#### BRIEF DESCRIPTION OF THE DRAWINGS

The present invention will be described with reference to the appended Figures, in which:

FIG. 1 is a schematic enlarged cross sectional view of the inventive underlayment used on a typical flat roof construction; and

FIG. 2 is a schematic cross section view of a typical flat roof system with the inventive underlayment;

These and other objects, advantages, and novel features of the present invention will become apparent when considered with the teachings contained in the detailed disclosure along with the accompanying drawings.

#### DESCRIPTION OF THE INVENTION

The present invention is directed toward a self-adhering water-resistant vapor permeable roofing underlayment membrane as shown in FIG. 1 which can be successfully used to cover flat and low sloped roofs ranging from about 0° to about 2° in slope as is shown in FIG. 2. Roofs from about 0° to about 5° can also be covered. The self-adhering roofing system is a UV stabilized, vapor permeable, water resistant, air barrier and is also rot proof and tear resistant. With vapor permeance ranging from about 25 perms to about 45 perms, most preferably about 35 perms, the underlayment membrane 10 allows the roof assembly to breathe or "dry out" as necessary during the seasonal changes. This helps to reduce or eliminate conditions that are conducive to mold, mildew, lumber distortion, insulation deterioration and metal corrosion. The drying aspect is of utmost importance in energy efficiency with single ply constructs in humid localities.

The present roof underlayment 10 as seen in FIG. 1 is constructed of permeable polyester sheet or membrane 12 of material ranging from about 180 mils to about 220 mils in thickness with a permeability ranging from about 65 perms to about 80 perms with a preferred permeability of about 75 perms. The polyester sheet 12 is premade and packaged in rolls which are unrolled at the manufacturing facility and coated at different stages. In some selected usages, permeable polypropylene can be used. The sheet of polyester which forms the substrate 12 of the underlayment 10 is coated with a permeable n-butyl acrylate copolymer coating 14 by a knife over roller in the first process stage.

The coating 14 is mixed prior to application on the polyester base layer and run through a foamer (high speed dispersion mixer) so that it formed with encapsulated air bubbles. These air bubbles are interconnected in the copolymer to form a permeable coating ranging from about 80 mils to about 100 mils in thickness with a permeability ranging from about 30 perms to about 60 perms when it is cured. The coating 14 is coated on the substrate 12 with a knife and roller in a wet application. The coating 14 is a wet foamed copolymer with the primary monopolymer being n-butyl acrylate mixed with another acrylate monopolymer.

Acrylates are the salts, esters and conjugate bases of acrylic acid and its derivatives. Acrylates contain vinyl groups; that is two carbon atoms double bonded to each other, directly attached to the carbonyl carbon.

Other polymers which can be mixed with the n-butyl acrylate are methyl acrylate, methyl methacrylate and

methyl acrylic acid. Carbon black at approximately 1% by weight of the copolymer solution is added to the copolymer. A suitable copolymer base coating is manufactured by BASF SE Corporation and sold under the trademark ACRONAL® 4250. This coating has a viscosity of 300 and a density (lb/gal of 8.6) with pH of about 7.7 with a temperature low point of -28° C.

The n-butyl acrylate polymer in the coating 14 ranges from 20 to 55% solids, with a pH ranging 7.7 to 8.0, and a preferred viscosity at 73° F. (cps) of 300 using a Brookfield RV viscometer Spindle #4 @ 100 rpm. The viscosity can effectively range from 100 to 500 depending on the percentage of solids. As previously noted, carbon black is also added to the copolymer to reduce tackiness, add strength and increase the UV effectiveness of the underlayment. The copolymer is foamed with a high speed dispersion mixer at 700 rpm with a 32% air injection with entrained air bubbles so that it has a foam density ranging from about 50% to about 65% preferably from about 55% to about 60%. The coating 14 is applied to the polyester substrate 12.

The coating 14 is then heat cured after leaving the coating blade setting the foamed air bubbles in place in the copolymer providing the coating with permeability. The coating 14 copolymer ranges from about 30% to about 98% n-butyl acrylate.

A copolymer pressure sensitive adhesive 16 is run through a second foamer so that it is formed with encapsulated air bubbles and is then applied to the cured acrylate coating 14 by a second blade coater, at a thickness ranging from about 4 mils to about 10 mils and cured as previously noted for the coating 14 to lock the air bubbles in place. Suitable pressure is applied to laminate the underlayment and the pressure sensitive adhesive has a preferred thickness of about 5 mils. The completed underlayment 10 has a permeability ranging from about 25 perms to about 45 perms and a preferred range from about 30 perms to about 40 perms.

The copolymer portion of the pressure sensitive adhesive (PSA) 16 has a backbone consisting of n-butyl acrylate, 2-ethylhexyl acrylate, and vinyl acetate. The structure of the backbone is shown in Table I below as follows:

TABLE I

(Structure of PSA Polymer Backbone)



The adhesive fully bonds to the coating 14 for air tightness and ease of installation and requires no primer for use on any substrate.

The pressure sensitive adhesive (PSA) is an acrylic solution. The polymeric portion of the PSA makes up at least 95% of the adhesive formulation and has a copolymer

backbone of n-butyl acrylate (about 60% by weight), 2-ethylhexyl acrylate (about 32% by weight) and vinyl acetate (about 7% by weight) forming a copolymer blend capable of bonding and crosslinking with the coating 14. Proper foaming of the adhesive is critical to good micropore formation. The aeration process includes high sheer mixing to entrain air in the mixed adhesive liquid solution. This is the same aeration process used for the coating. The self-adhering adhesive 16 is evenly applied on the n-butyl acrylate coating, cured and the micropores are formed and fixed throughout the PSA. The coating method used with the present invention for both the coating 14 and the PVA 16 was accomplished with a blade coater. This is a non-contact coating method and it does not crush or destroy the foam in the copolymer during coating. After application, the adhesive must be heated to lock-in the micropore formation. The adhesive in the present invention was reformulated by adding surfactants and water to the copolymer to control bubble size, bubble density, viscosity, and stability of the copolymer. The peel value of the adhesive is reduced by the introduction of voids (air bubbles) and the addition of carbon black and a surfactant such as long chain alcohols create a stable inverse emulsion.

The acrylate polymer coating 14 does not require a slip sheet when applied. It is dry enough to be rolled onto itself. The pressure sensitive adhesive 16 is applied to a siliconized release film 17 and then laminated to the polyester and coating composite.

Microscopy of the modified adhesive surface was performed revealing a porous structure of the adhesive having a bubble density (number of pores) ranging from about 4000 pores in 1.0 in<sup>2</sup> to about 4600 pores in 1.0 in<sup>2</sup>, preferably about 4400 pores in 1.0 in<sup>2</sup> with a majority of the pores, preferably about 80% to about 90% of the bubbles/pores having a size ranging from about 200 microns to about 300 microns. The pores formed are generally round and oval in shape and form a vapor pathway through the adhesive layer. The majority of the pores 100 formed by the bubbles appear to be distributed evenly across the surface penetrating through the adhesive layer when the polymer mixture is heat treated to set the pores in the adhesive. Preferably, the density of the foamed adhesive should fall between about 0.65 and about 0.75 after aeration.

The adhesive copolymer which was manufactured and as shown in Table I ranges from about 45% by weight to about 50% by weight, preferably about 48% to about 49% by weight. The copolymer was mixed with a first solvent-free, surfactant-based wetting agent, preferably ranging from about 4% by weight to about 6% by weight, and most preferably about 5% by weight to provide emulsification and bubble size; and a second surfactant such as a foaming agent ranging from about 1.5% by weight to about 2.0% by weight, and preferably about 1.7% by weight to provide foam formation. A polymeric based thickener was added to the mixture in a range from about 0.2% by weight to about 0.4% by weight, preferably about 0.30% by weight. The adhesive copolymer composition was added to water ranging from about 40% by weight to about 50% by weight, preferably about 43% by weight to about 45% by weight and mixed in a high speed dispersion mixer at 500 rpm to form uniform bubbles in the mixture and fed into a coater feeder as previously described. The foamed adhesive was coated onto the cured porous n-butyl acrylate coating and heat cured to form the pores in place in the copolymer. The pressure sensitive adhesive and underlayment is laminated to reduce tackiness of the pressure sensitive adhesive and the need for a slip sheet.

For industry testing standards, the present underlayment 10 will support a water column of twenty four (24) inches of water for forty eight (48) hours.

Construction of a typical roof composite for a commercial 5 flat roof 20 using the underlayment is shown in FIG. 2. In FIG. 2, a typical construction of a flat composite deck roof deck 21 using the inventive underlayment 10 which allows for drying of the roof composite from the inside out is shown. In this embodiment, a ½ inch mechanically attached 10 thermal barrier board 24 fastened to the metal roof deck 22 by mechanical fasteners such as screws or nails 23. The permeable membrane underlayment 10 of the present invention is mounted on the barrier board 24 and secured thereto by the pressure sensitive adhesive 16. Two layers of polyiso 15 26, 3 inches and 2.2 inches, (5.2 inches total), thickness as needed for insulation value, are set in low rise foam adhesive 27. A ½ inch cover board 28 is set in low rise foam adhesive 27 which has been layered on the top polyiso layer 26 and the roof is covered with a PVC, or other single ply roof 20 membrane 29 which is also set in low rise foam adhesive 27.

The principles, preferred embodiments and modes of operation of the present invention have been described in the foregoing specification. However, the invention should not be construed as limited to the particular embodiments which have been described above. Instead, the embodiments described here should be regarded as illustrative rather than restrictive. Variations and changes may be made by others without departing from the scope of the present invention as defined by the following claims:

30 What is claimed is:

1. An underlayment for a roof having a slope angle of 5° or less, that is an air barrier and self-adhering, vapor-permeable, water-resistive, and UV-resistant, the underlayment comprising:

a substrate of polyester having a surface;  
a foamed, permeable copolymer coating attached to the polyester substrate's surface, wherein the foamed, permeable copolymer coating includes an n-butyl acrylate copolymer that;  
includes n-butyl acrylate in an amount ranging from 30% to 98% by weight, and  
has a foam density that ranges from 50% to 65% of the copolymer's density before foaming; and  
a permeable pressure-sensitive adhesive bonded to said foamed,  
permeable copolymer coating; the underlayment having a permeability of 25 perms or more.

2. The underlayment as claimed in claim 1, wherein the underlayment has a permeability of about 35 perms or more.

3. The underlayment as claimed in claim 1, wherein the permeable-pressure-sensitive adhesive does not include a solvent.

4. The underlayment as claimed in claim 1, wherein the foamed, permeable copolymer coating includes n-butyl acrylate copolymer with solids ranging from about 30% to about 55% of the foamed, permeable copolymer coating.

5. The underlayment as claimed in claim 1, wherein the foamed permeable copolymer coating has a permeability that ranges from about 30 perms to about 60 perms.

6. The underlayment as claimed in claim 1, wherein the polyester substrate ranges in thickness from about 180 mils to about 220 mils, and has a permeability that ranges from about 65 perms to about 80 perms.

7. The underlayment as claimed in claim 1, wherein the foamed permeable copolymer coating includes carbon black.

**8.** A membrane for a flat or low sloped roof, that is an air barrier, and water-resistant, vapor-permeable, and self-adhering, the membrane comprising:

- a substrate of polyester having a surface, and that is permeable and consists of a single ply;
  - a foamed, permeable n-butyl acrylate copolymer coating attached to the polyester substrate's surface, comprising n-butyl acrylate copolymer, wherein the n-butyl acrylate copolymer has a foam density that ranges from 50% to 65% of the n-butyl acrylate copolymer's density before foaming;
  - a pressure-sensitive, permeable, co-polymer acrylate adhesive bonded with the foamed, permeable n-butyl acrylate copolymer coating; and
- wherein, the combination of the substrate, the foamed, permeable n-butyl acrylate copolymer coating, and the pressure-sensitive, permeable copolymer acrylate adhesive has a permeability that ranges from about 25 perms to about 45 perms.

**9.** The membrane of claim **8** wherein said low sloped roof has a sloped angle of 5° or less.

**10.** The membrane of claim **8** wherein the pressure-sensitive, permeable, copolymer acrylate adhesive includes a silicon release film.

**11.** The membrane as claimed in claim **8** wherein the foamed, permeable n-butyl acrylate copolymer coating includes carbon black.

**12.** The membrane of claim **8** wherein the foamed, permeable n-butyl acrylate copolymer includes solids ranging from about 20% to about 50%.

**13.** The membrane of claim **8** wherein the pressure-sensitive, permeable, copolymer acrylate adhesive includes

a removable silicon release film mounted thereto to form an exterior surface of said roofing membrane.

**14.** A membrane laminate for a flat roof, that is an air barrier and water-resistant, UV-resistant, vapor-permeable, and self-adhering, the laminate comprising:

- a substrate of polyester having a surface and that is vapor permeable;
- a foamed, vapor-permeable, solvent-free, n-butyl acrylate copolymer coating attached to the polyester substrate's surface, wherein the foamed, vapor-permeable, solvent-free, n-butyl acrylate copolymer coating includes carbon black;
- a permeable, pressure-sensitive, copolymer adhesive attached to the foamed, vapor-permeable, solvent-free, n-butyl acrylate copolymer coating, wherein the permeable, pressure-sensitive, copolymer adhesive is vapor permeable; and

wherein the combination of the substrate, the foamed, vapor-permeable, solvent-free, n-butyl acrylate copolymer coating, and the permeable, pressure-sensitive, copolymer adhesive has a permeability greater than 25 perms.

**15.** The membrane laminate as claimed in claim **14** wherein the foamed, vapor-permeable, solvent-free, n-butyl acrylate copolymer coating has a thickness ranging from about 80 mils to about 100 mils.

**16.** The membrane laminate as claimed in claim **14** wherein the membrane laminate is capable of supporting a water column at least 24 inches high for at least 48 hours.

\* \* \* \* \*